

## UNITED STATES PATENT OFFICE

2,596,705

## MAGNETIC ALLOY

Donald L. Martin, Ballston Lake, N. Y., assignor  
to General Electric Company, a corporation of  
New York

No Drawing. Application September 27, 1950,  
Serial No. 187,157

6 Claims. (Cl. 75—134)

1

The present invention relates to a new and improved magnetic alloy. More specifically it is concerned with a magnetic alloy particularly useful in the fabrication of rotors for hysteresis motors.

A hysteresis motor may be defined as a type of synchronous motor without D. C. excitation, which starts by virtue of the hysteresis losses induced in the rotor by the revolving magnetic field of the primary and operates normally at synchronous speed due to the magnetic retentivity of the rotor member. A typical rotor construction is shown in Patent 1,768,386—Warren as comprising a continuous ring of magnetic material provided with an integral bar or bars across the diameter. The ring cooperates with a rotating magnetic field to produce the starting torque and the bar or bars produce a polar synchronizing effect to bring the rotor into and hold it in synchronism. In the construction shown in the Warren patent, the bar also serves as a spider for supporting the rotor member on the motor shaft.

In an "ideal" hysteresis motor, the hysteresis torque is constant at all speeds from standstill to synchronism. In other words the starting torque, pull-in torque and pull-out torque are all mutually equal to one another. In practice, however, it has not been possible to attain these ideal conditions or even to approach them with the types of rotor materials presently available.

The present invention has its principal object the provision of an improved magnetic alloy particularly adapted for the manufacture of hysteresis motor rotors.

A further object of the invention is to provide a cold workable and heat treatable magnetic alloy characterized by a high residual induction  $B_r$  and a medium coercive force  $H_c$  in the range of from 50 to 100 oersteds.

It has been found that these objects can be attained with an alloy essentially comprising 43 to 47 percent by weight cobalt, 4 to 6 percent vanadium and 5 to 7 percent nickel, balance iron except for incidental impurities. A preferred alloy is one containing 45.6% cobalt, 4.4% vana-

2

dium and 6.1% nickel, balance iron. These alloys are characterized by good cold workability combined with a relatively high  $B_r/H_c$  ratio and a coercive force between 50 and 100 oersteds.

5 Nickel within the critical range of from 5 to 7 percent is an essential component of the present alloy and distinguishes it both magnetically and from the standpoint of composition from known cobalt-iron-vanadium alloys such as the alloy described in Patent 1,862,559—White et al. With these critical amounts of nickel and by holding the vanadium content of the alloy within the prescribed limits, preferably about 4.4% by weight, there is obtained a cold workable alloy 15 which can be readily rolled to thicknesses as small as 0.010" to provide a sheet or strip suitable for use in the stamping of hysteresis motor rotor laminations, which cold rolled material by a suitable heat treatment can be given magnetic 20 properties including a residual induction of at least 12,000 gauss usually at least 14,000 gauss, and a coercive force of from 50 to 100 oersted.

In the practice of the present invention a melt of the four ingredients in the specified proportions is cast and the casting subjected to an elevated temperature of about 1000° C. for a period of time before hot rolling to a thickness of about 0.1 inch. The brittle material obtained at this thickness is then annealed at about 1000° C. and water quenched prior to cold rolling to a finish thickness of about 10 mils. Rotor laminations are punched from the cold rolled strip.

To develop the desired magnetic qualities, the resultant punchings are heat treated for a period of from 15 minutes up to an hour or more at a temperature in the neighborhood of 600° C. After heat treatment rotor laminations of an alloy of 45.6% cobalt, 6.1% nickel, 4.4% vanadium, balance iron except for incidental impurities exhibited  $B_r$  of 14,100 gauss and  $H_c$  of 90 oersteds and  $B_d$   $H_d$  Max of 605,000. These rotor members assembled into a standard hysteresis motor were torque tested and compared with a similar rotor composed of the magnetic material 40 currently employed for this purpose and known as a 5% tungsten steel.

| Alloy              | Pull Out <sup>1</sup> | At 115v.<br>Stall | Start | Pull In | Pull Out | At 92v.<br>Stall | Start | Pull In |
|--------------------|-----------------------|-------------------|-------|---------|----------|------------------|-------|---------|
| P6                 | 1.94                  | 1.94              | 1.39  | 1.33    | 1.21     | 1.41             | 1.07  | 1.00    |
| Sandvik<br>5.75% W | 1.62                  | 1.62              | 0.76  | 0.75    | 1.16     | 1.16             | 0.57  | 0.57    |

<sup>1</sup> Pull Out is maximum torque at synchronous speed. Stall is stalling torque. Start is starting torque at non-synchronous speed. Pull In is starting torque at synchronous speed.

In the above table, the alloy of the present invention is designated as P6 and the currently used standard alloy as a 5.75% tungsten having a Br of about 10,500 and an H<sub>c</sub> of about 60. The actual composition of the tungsten alloy is 5.75% tungsten, 0.68 carbon, 0.40 chromium, balance iron.

From the results set forth in this table, it will be seen that the alloy of the present invention provides higher torque values under all test conditions. It is also apparent that a hysteresis motor comprising the alloy of the present invention approaches much more nearly the requirements of an ideal hysteresis motor. For example whereas the pull-out torque for the motor containing the tungsten steel rotor is more than twice the starting torque or the pull-in torque at 115 volts, the motor equipped with the alloy of the present invention had a pull-out torque which was only about 35% higher than the starting and pull-in torques. At 92 volts the motor having a rotor composed of the alloy of the present invention is characterized by pull-out starting and pull-in torques which were substantially the same.

These differences between the alloy of the present invention and the standard Sandvik alloy are attributable at least in part to the differences in their Br/H<sub>c</sub> ratios. The alloy of the present invention while being characterized by approximately the same coercive force has a Br value at least 2500 gauss higher than the tungsten steel.

What I claim as new and desire to secure by Letters Patent of the United States is:

1. A magnetic alloy comprising 5 to 7 percent nickel, 4 to 6 percent vanadium, 43 to 47 percent cobalt, balance substantially all iron, said alloy having a coercive force between 50 and 100 oersteds and a Br of at least 12,000 gauss.

2. A cold workable magnetic alloy comprising 5 to 7 percent nickel, 4 to 6 percent vanadium, 43 to 47 percent cobalt, balance substantially all iron except for incidental impurities.

10 3. The alloy of claim 1 containing 6.1% nickel, 4.4% vanadium, 45.6% cobalt, balance iron.

4. The alloy of claim 2 containing 6.1% nickel, 4.4% vanadium and 45.6% cobalt.

5. A rotor lamination for a hysteresis motor 15 composed of the cold worked and heat treated alloy of claim 1.

6. A rotor lamination for a hysteresis motor composed of the cold worked and heat treated alloy of claim 3.

20 DONALD L. MARTIN.

#### REFERENCES CITED

The following references are of record in the file of this patent:

25 UNITED STATES PATENTS

| Number    | Name  | Date          |
|-----------|-------|---------------|
| 1,862,559 | White | June 14, 1932 |

50 OTHER REFERENCES

Transactions A. I. M. E., vol. 188, February 1950, Journal of Metals. Published by the A. I. M. E., New York. Pages 287, 291, 292 and 293.